

Feb. 16, 1937.

A. G. PETERKIN, JR.

2,070,680

## PROCESS OF CONVERTING HYDROCARBON OILS

Filed Nov. 21, 1923



Inventor:  
Albert G. Petersen Jr  
By Cornelius L. Schut  
his Attorney.

## UNITED STATES PATENT OFFICE

2,070,680

## PROCESS OF CONVERTING HYDROCARBON OILS

Albert G. Peterkin, Jr., Bryn Mawr, Pa., assignor to The Atlantic Refining Company, Philadelphia, Pa., a corporation of Pennsylvania

Application November 21, 1928, Serial No. 320,778

8 Claims. (CL 196—58)

My invention relates to conversion or cracking of high boiling point hydrocarbon oils, particularly petroleum or components thereof, to produce lower boiling point oils suitable for use as motor fuels in internal combustion engines, with particular reference to the cracking of oils of high specific gravity, more particularly residual oils resulting from cracking or noncracking distillations.

10 In accordance with my invention, oils of such high boiling point, high specific gravity and objectionable solid content or other properties which render it difficult and relatively costly to process them in usual cracking systems, are converted or cracked with relative ease and at comparatively low cost to form solid coke, suitable for use as fuel, lower boiling oil suitable for motor fuel or for further cracking to produce motor fuel, and gas which may be burned or used for the production of the higher alcohols and other compounds.

20 In cracking processes, in which the oil to be converted into lower boiling components is passed through a heated tubular passage, there is formed heavy carbonaceous material which tends to adhere to the tube walls and form coke deposits which impair heat transfer to the oil and may induce damage to the tubes, and which must be removed from time to time. Such deposit of carbon occurs more readily with heavy residual oils which tend to form greater quantities of carbonaceous material. For this reason cracking processes are generally practiced on distillates, as gas oil.

30 The heavy oils, as residues from a cracking or noncracking distillation, and high boiling crude oils, may be cracked by maintaining the heating tubes at a relatively low cracking temperature so that mild cracking occurs with relatively low concentration of heavy carbonaceous material and with consequent less tendency for the carbonaceous material to adhere to the tube walls. This is an inefficient method, however, due to the low yields of low boiling oils or gasoline obtained. Another mode of operation is to admix with the residual oil a diluent, as gas oil, produced in the process and/or from an outside source, which reduces the concentration of heavy carbonaceous products and hence reduces carbon formation. The proportion of diluent required is however relatively too high for economical operation and may require a source of gas oil in addition to the residual oil to be cracked.

40 My invention relates to improvements in cracking processes whereby heavy oils, as for example 10° to 20° A. P. I. bottoms from distillation of crude petroleum, residuum from a cracking

operation, or heavy crude petroleum, may be economically cracked without dilution and without substantial carbon deposition on the walls of the heating tubes, thereby eliminating the necessity for cleaning and reducing replacements of 5 the tubes.

In accordance with my invention this result is attained by bringing the oil to the temperature of incipient cracking and immediately introducing it into a coking chamber, preferably not externally or separately heated, where the oil is maintained at elevated temperature to permit its cracking to form volatile products, which leave the chamber as vapors, and coke which is deposited therein out of contact with externally 10 heated surfaces.

More particularly in accordance with my invention, the residual oil is brought to the temperature of incipient cracking by passage through a heating zone at such high velocity that substantially no cracking occurs due to the relatively short time the oil is subjected to cracking temperature. The oil so heated is discharged into a coking chamber where it is maintained at cracking temperature, due either solely to the 20 heat absorbed while in the aforesaid heating zone or to additional heat of cracked products introduced into the coking chamber from a second heating zone operated at a higher temperature. In the coking chamber there is effected cracking 25 of the residual oil into coke, gas, and lower boiling hydrocarbons, portions of which have a 30 boiling point too high to be suitable for gasoline or motor fuel, and which pass as vapors from the coking chamber into suitable dephlegmating equipment where they are condensed and 35 passed to the aforesaid second heating zone wherein substantial cracking occurs and the highly heated cracked products, hydrocarbons of still lower boiling point, as gasoline, thus 40 formed are introduced into the coking chamber.

45 For an understanding of my invention reference may be had to the accompanying drawing illustrating diagrammatically one form of apparatus suitable for practicing my process.

In the drawing, A is a furnace heated by the burner 1 and containing the pipe coil 2 fed by the pump 3. B is a coking chamber, preferably heat insulated by covering 6, into which the coil 2 discharges through line 4. C is a fractionating 50 column into which the vapor from the coking chamber B is discharged through line 5. D is a partial condenser, in communication with the column C through the vapor line 6, from which the line 7 leads to the condenser E which in turn 55

is connected by the line 9 to the gas separator F. From the gas separator the line 10, controlled by valve 10a, leads to suitable gas storage while the line 11 controlled by valve 11a leads to liquid storage.

From the bottom of the column C the line 8, in which is the pump 12, leads to the coil 13 in the second furnace G or heating zone, heated by the burner 14. The line 15, in which is the pressure reducing valve 15a, leads to and preferably extends to a point near the bottom of, the chamber B. Line 16 leads from an external supply of gas oil to the line 8.

In the operation of the process, residual oil, for example bottoms from the noncracking distillation of Midcontinent crude petroleum and having a gravity of 12° in the A. P. I. scale, is fed by the pump 3 through the coil 2 wherein the oil is heated to the temperature of incipient cracking, for example 800° F., and immediately, or before substantial cracking occurs, is discharged through the line 4 into the coking chamber B. The rate of cracking is primarily dependent upon the temperature of the oil and when the oil is at a relatively low temperature the rate of cracking is correspondingly low and therefore little or no cracking occurs in the tubes 2. Within the chamber B is maintained a relatively low pressure, for example 30 pounds per sq. in. gauge, and the pressure drop in the tubes 2 is preferably only sufficient to effect passage of the oil therethrough at suitably high rate. Tubes 2 are not primarily cracking tubes; they merely heat the heavy oil to the cracking temperature.

In the chamber B the oil is maintained at cracking temperature, attained in tubes 2, or supplemented by heat of or from the highly heated cracked products introduced into chamber B through line 15 from the coil 13 in which occurs substantial cracking as hereinafter described. The maintenance of the residual oil at the cracking temperature effects its conversion while in the coking chamber B into lower boiling hydrocarbons, gas and solid coke. The gas and vapors of the lower boiling hydrocarbons, together with the cracked vapors introduced through the line 15, pass through line 5 into the fractionating column C where they are passed countercurrent to descending reflux liquid, formed by condensation in the partial condenser D of a portion of the vapors leaving column C. As a result of the fractionation the higher boiling portion of the vapors is condensed in the column while the lower boiling portion passes as a vapor with the gases to the condenser E in which it is cooled and forms a liquid condensate suitable for use as or in production of motor fuel. The other portion, withdrawn as liquid from the bottom of the column C through line 8, has a boiling range too high for use as gasoline and has in general the characteristics of gas oil.

The condensate from the condenser E is passed with the uncondensed gas to the separator F from which the gas and liquid are separately withdrawn through the lines 10 and 11, respectively, and passed to storage or otherwise suitably disposed of or treated.

The high boiling fraction withdrawn through the line 8 requires further cracking to cause conversion into compounds, such as gasoline, of suitably low boiling point. Since this high boiling fraction is a distillate, carbon deposition will take place much less readily during cracking

than would occur in the cracking of the heavy residual oil heated in the coil 2. Therefore this oil is fed by pump 12 through line 8 to the tubes 13 in which substantial cracking is effected by bringing it to an elevated temperature, for example 90° F., while under a high pressure, for example 850 pounds per sq. in. gauge. The length of the tubes, the pressure and the velocity are so adjusted or related that the oil is maintained under cracking conditions in the coil 13 for a sufficient period of time to permit substantial cracking with formation of appreciable quantities of practical or commercial yields of gasoline-like products. If desired additional quantities of charging stock suitable for high temperature cracking, as gas oil or other distillate of boiling point higher than that of gasoline, may be fed through line 16 to line 8 and thence to coil 13.

The highly heated cracked products are discharged through the pressure reducing valve 15a into the low pressure coking chamber B, preferably beneath the surface of the hot residual oil. It is not essential that the cracked products introduced at high temperature into the coking chamber pass through the residual oil; they may, for example, be introduced into the space above the liquid oil. The introduction of this hot material from tubes 13 maintains the residual liquid oil at cracking temperature or may serve further to increase its temperature thereby causing cracking of the residual oil to occur at an increased rate. As a result the coke resulting from cracking of the heavy oil is formed in the coking chamber B, unheated except by the oils introduced into it, where it is deposited out of contact with heated surfaces.

It will thus be seen that the residual oil is cracked to form products the major portion of which are not suitable for motor fuel but are suitable as charging stock for a high temperature, high pressure cracking system in which relatively high yields of gasoline-like products are formed; and the excess heat in these cracked products is utilized to maintain or increase the temperature of the hot residual liquid oil so that there are obtained additional quantities of charging stock for the more severe cracking in tubes 13. The ultimate products from the treatment of the residual oil are coke, motor fuel and gas.

The more or less diagrammatic illustration of the apparatus is for purposes of description, and does not show details, such as structural modifications or features which are apparent to one skilled in this art.

Although only one coking chamber is shown, it shall be understood that a second chamber may be put into operation during removal of coke from the other chamber.

It shall be understood that the system G, 13 generically represents any suitable method or system for cracking oil, whose reaction products may be introduced into coking chamber B, as herein described and preferred, or separately disposed of or further treated. My invention is therefore not limited to the particular mode described of cracking the high boiling distillate recovered from the fractionating column. For example, the cracked products from the tubes 13 may be passed through intermediate apparatus for further treatment of any kind, including cracking, before passage to the coking chamber B. Or the pressure reducing valve 15a may be omitted and the tubes 13 be maintained under the pressure existing in the coking chamber B.

in which may be maintained atmospheric or any suitable superatmospheric pressure.

While my invention has been described by ad-  
5 versions to particular temperatures and pressures,  
it is not to be limited to these conditions which,  
while comprehended in my invention, are speci-  
fied merely for purpose of illustration. The tem-  
perature of the heating tubes 2 should be suffi-  
10 cient to bring the heavy oil to substantially the  
cracking temperature for example, 650° to 800°  
F., while the pressure may be merely that re-  
quired to force the oil through the tubes, or a  
superatmospheric pressure of any suitable mag-  
nitude may be maintained in the coking chamber  
15 B. The high temperature cracking coil 13 is  
maintained at temperatures in excess of 800° F.  
and the cracking effected in the liquid phase, un-  
der high pressure, as in excess of 100 pounds per  
square inch, or in vapor phase under lower pres-  
20 sure.

From the foregoing description it will be per-  
ceived that in one of its aspects my invention  
comprises a cracking system, including a crack-  
ing zone, such as a coking chamber B, in which  
25 occurs substantially all the cracking of the oil  
previously elevated to cracking temperature in a  
heating zone, as in heat-absorption structure 2,  
with production in the cracking zone of coke,  
lower boiling oils and gas.

30 In another of its aspects my invention com-  
prises two co-operative cracking systems, one of  
them as aforesaid, and the second, operating to  
crack a lower boiling oil, either derived from a  
separate source, an oil from the first cracking  
35 system, or the combination of the latter with oil  
from a separate source, with delivery of products  
from the second cracking system into the crack-  
ing zone or coking chamber of the first system.

For brevity in the appended claims the term  
40 "residual oil" refers to oil operated upon in the  
first cracking system and includes heavy oils of  
the character herein defined by that term; the  
term "intermediate boiling point" is employed  
generically to designate the oil charged into the  
45 second cracking system; and the term "low boil-  
ing point" is employed generically to designate  
oil constituting an ultimate product, such as  
cracked naphtha, gasoline or other oils of lower  
boiling point than that of the oil charged into  
50 the second cracking system.

What I claim is:

1. A hydrocarbon oil cracking process which  
comprises passing the oil in a restricted stream  
through a heating zone and heating the same  
55 therein to cracking temperature under sufficient  
pressure to maintain a substantial portion there-  
of in the liquid phase, discharging the heated oil  
into a separating zone and separating the same  
into vapors and unvaporized oil therein, simul-  
60 taneously heating hydrocarbon vapors to vapor  
phase cracking temperature in a second heating  
zone maintained at higher temperature than the  
first-mentioned heating zone, and injecting re-  
sultant vapor phase cracked vapors from said  
65 second zone in amount and at a temperature  
sufficient to distill the unvaporized oil to coke.

2. In coking hydrocarbon oils, the improve-  
ment which comprises supplying a hydrocarbon  
oil to a vapor phase cracking operation, vaporiz-  
70 ing and cracking the oil in the vapor phase there-  
in, releasing the hot vapor mixture from the  
vapor phase cracking operation at a temperature  
upwards of 900° F. within a coking receptacle,  
heating a heavy hydrocarbon oil to be coked to  
75 a temperature upwards of 700° F. by supplying

heat thereto from an extraneous source in a  
heating zone separate from the heating zone  
used in the vapor phase cracking operation, in-  
troducing the thus preheated heavy oil into the  
coking receptacle into direct contact with the  
hot vapor mixture discharged from the vapor  
phase cracking operation, and thereby reducing  
said heavy oil to coke therein.

3. In coking heavy hydrocarbon oils, the im-  
provement which comprises heating the heavy 10  
oil stock to be coked to a temperature upwards  
of 700° F. in a heating zone by supplying heat  
from an extraneous source and introducing the  
thus preheated stock into a coking receptacle,  
and heating a fluid coking medium to a tempera-  
15 ture upwards of 900° F. in a separate heating zone  
by supplying heat from an extraneous source  
and releasing the thus heated coking medium  
within the coking receptacle and thereby reduc-  
ing said stock to coke in the coking receptacle. 20

4. In coking heavy hydrocarbon oils, the im-  
provement which comprises heating the heavy oil  
stock to be coked to a temperature as high as  
25 800° F. in a heating zone by supplying heat from  
an extraneous source and introducing the thus  
preheated stock into a coking receptacle, and  
heating a fluid coking medium to a temperature  
upwards of 900° F. in a separate heating zone by  
30 supplying heat from an extraneous source and  
releasing the thus heated coking medium within  
the coking receptacle and thereby reducing said  
stock to coke in the coking receptacle.

5. In coking tars from cracking operations for  
the production of gasoline, the improvement  
35 which comprises heating the tar to a temperature  
upwards of 700° F. in a heating zone by supply-  
ing heat thereto from an extraneous source and  
introducing the thus preheated tar into a coking  
receptacle, and heating a fluid coking medium  
40 to a temperature upwards of 900° F. by supplying  
heat thereto from an extraneous source in a heating  
zone separate from the first mentioned heating  
zone and releasing the thus superheated coking  
medium within the coking receptacle, and  
45 thereby reducing the tar to coke in the coking  
receptacle.

6. The method of converting high boiling hy-  
drocarbon oils into lower boiling products and  
50 a coke residue which comprises, continuously  
flowing a stream of oil consisting substantially  
entirely of heavy oil residues once through an  
elongated heated passageway while heating said  
stream to a cracking temperature, discharging  
55 the stream of hot products into the lower portion  
of an enlarged chamber wherein unvaporized  
constituents of said stream are collected and  
caused to decompose to a substantially solid coke  
residue, simultaneously flowing a stream of oil  
60 consisting substantially entirely of distillate oil  
stock through an independent heated passageway  
while heating the said stream to a temperature  
of at least 900° F. to effect conversion thereof  
into desired low boiling products, discharging the  
65 latter separate stream of highly heated cracked  
products into said enlarged chamber substantial-  
ly below the point of introduction of the heavy  
oil residues wherein they enter into the said mass  
of residue below the level thereof and thus im-  
part heat thereto to further the decomposition  
70 of said residues into coke, separately withdraw-  
ing vapors from said enlarged chamber and sub-  
jecting them to fractionation to condense as re-  
flux condensate undesired higher boiling constit-  
uents thereof, withdrawing and condensing the  
75

35

40

45

50

55

60

65

70

75

fractionated vapors, and separately withdrawing reflux condensate from said fractionating zone and passing it to said last named heated passageway as distillate charging stock therefor while avoiding passage of any of the said residues from said enlarged chamber to either of said heated passageways.

7. A combined cracking and coking process for converting a hydrocarbon oil residue into coke and light distillate, which comprises heating a continuous confined stream of such residue in a furnace to a cracking temperature while causing said stream to move at a sufficiently rapid rate to prevent substantial cracking, discharging the heated stream without substantial reduction of pressure into the lower portion of an enlarged chamber, removing only vaporous products from the chamber while retaining the liquid constituents therein and maintaining the mass in the chamber at a coking temperature substantially entirely by reason of the heated products discharged thereinto to thereby effect conversion into a coke residue, condensing the higher boiling portion of the vapors removed from said chamber, heating the resulting condensate while in transit through a separate furnace to a temperature of at least 900° F. to effect conversion of said condensate into lower boiling oils and introducing the heated condensate into said

chamber substantially below the point of introduction of said oil residue wherein they enter into the said mass of residue below the level thereof, and condensing the relatively low boiling constituents of said vapors to form a light 5 distillate.

8. The process of converting high boiling hydrocarbon oils into lower boiling ones which comprises continuously passing the higher boiling hydrocarbon oil through a heating zone in which 10 it is raised to a cracking temperature without therein undergoing substantial cracking, passing the oil thus heated into the lower portion of a coking zone where distillation takes place, removing evolved vapors from the coking zone while 15 retaining the liquid therein, maintaining the mass in the coking chamber to thereby convert the same to a coke residue, condensing the higher boiling portion of the vapors removed from the coking zone, heating the resulting condensate 20 during passage through a separate heating zone to a temperature of at least 900° F. and continuously introducing the heated condensate into said coking zone substantially below the point of introduction of the higher boiling hydrocarbon oil 25 wherein they enter into the liquid retained in the coking chamber below the level thereof and thus impart additional heat thereto.

ALBERT G. PETERKIN, JR.

CERTIFICATE OF CORRECTION.

Patent No. 2,070,680.

February 16, 1937.

ALBERT G. PETERKIN, JR.

It is hereby certified that error appears in the above numbered patent requiring correction as follows: In the heading to the drawing, line 3, for the filing date "Nov. 21, 1923" read Nov. 21, 1928; page 2, second column, line 6, for "90° F." read 920° F.; and that the said Letters Patent should be read with these corrections therein that the same may conform to the record of the case in the Patent Office.

Signed and sealed this 20th day of April, A. D. 1937.

(Seal)

Henry Van Arsdale  
Acting Commissioner of Patents.

fractionated vapors, and separately withdrawing reflux condensate from said fractionating zone and passing it to said last named heated passageway as distillate charging stock therefor while avoiding passage of any of the said residues from said enlarged chamber to either of said heated passageways.

7. A combined cracking and coking process for converting a hydrocarbon oil residue into coke and light distillate, which comprises heating a continuous confined stream of such residue in a furnace to a cracking temperature while causing said stream to move at a sufficiently rapid rate to prevent substantial cracking, discharging the heated stream without substantial reduction of pressure into the lower portion of an enlarged chamber, removing only vaporous products from the chamber while retaining the liquid constituents therein and maintaining the mass in the chamber at a coking temperature substantially entirely by reason of the heated products discharged thereinto to thereby effect conversion into a coke residue, condensing the higher boiling portion of the vapors removed from said chamber, heating the resulting condensate while in transit through a separate furnace to a temperature of at least 900° F. to effect conversion of said condensate into lower boiling oils and introducing the heated condensate into said

chamber substantially below the point of introduction of said oil residue wherein they enter into the said mass of residue below the level thereof, and condensing the relatively low boiling constituents of said vapors to form a light 5 distillate.

8. The process of converting high boiling hydrocarbon oils into lower boiling ones which comprises continuously passing the higher boiling hydrocarbon oil through a heating zone in which 10 it is raised to a cracking temperature without therein undergoing substantial cracking, passing the oil thus heated into the lower portion of a coking zone where distillation takes place, removing evolved vapors from the coking zone while 15 retaining the liquid therein, maintaining the mass in the coking chamber to thereby convert the same to a coke residue, condensing the higher boiling portion of the vapors removed from the coking zone, heating the resulting condensate 20 during passage through a separate heating zone to a temperature of at least 900° F. and continuously introducing the heated condensate into said coking zone substantially below the point of introduction of the higher boiling hydrocarbon oil 25 wherein they enter into the liquid retained in the coking chamber below the level thereof and thus impart additional heat thereto.

ALBERT G. PETERKIN, JR.

CERTIFICATE OF CORRECTION.

Patent No. 2,070,680.

February 16, 1937.

ALBERT G. PETERKIN, JR.

It is hereby certified that error appears in the above numbered patent requiring correction as follows: In the heading to the drawing, line 3, for the filing date "Nov. 21, 1923" read Nov. 21, 1928; page 2, second column, line 6, for "90° F." read 920° F.; and that the said Letters Patent should be read with these corrections therein that the same may conform to the record of the case in the Patent Office.

Signed and sealed this 20th day of April, A. D. 1937.

(Seal)

Henry Van Arsdale  
Acting Commissioner of Patents.

CERTIFICATE OF CORRECTION.

Patent No. 2,070,680.

February 16, 1937.

ALBERT G. PETERKIN, JR.

It is hereby certified that error appears in the above numbered patent requiring correction as follows: In the heading to the drawing, line 3, for the filing date "Nov. 21, 1923" read Nov. 21, 1928; page 2, second column, line 6, for "90° F." read 920° F.; and that the said Letters Patent should be read with these corrections therein that the same may conform to the record of the case in the Patent Office.

Signed and sealed this 20th day of April, A. D. 1937.

(Seal)

Henry Van Arsdale  
Acting Commissioner of Patents.